

# United States Patent

[11] 3,615,896

[72] Inventors Arthur J. Berger  
Croton-on-Hudson;  
Albert W. Cizek, Jr., Valley Stream;  
Raymond J. Simeon, Middleburg, all of  
N.Y.  
[21] Appl. No. 846,418  
[22] Filed July 31, 1969  
[45] Patented Oct. 26, 1971  
[73] Assignee The United States of America as  
represented by the Secretary of the Navy

[56] References Cited  
FOREIGN PATENTS  
1,147,820 4/1963 Germany..... 148/6.16  
Primary Examiner—Ralph S. Kendall  
Attorneys—Louis A. Miller, Louis B. Applebaum and Philip  
Schneider

[54] METAL SURFACE PRIMER  
4 Claims, 1 Drawing Fig.

[52] U.S. Cl..... 148/6.16,  
117/75, 260/292.2 TN  
[51] Int. Cl..... C23f 7/10  
[50] Field of Search..... 117/161  
KP, 75; 260/292.2 TN, 29.2 M, 29.6 M; 148/6.16,  
6.2, 6.15

**ABSTRACT:** A deck primer for use with nonslip deck  
coatings of the chemically cured-resin type comprising a mix-  
ture of Formula No. 117 wash primer (as set forth in Military  
Specification MIL-D-23003(SHIPS) and its Amendment 2) and a specific, moisture-cured, polyurethane resin, in the ratio  
of 5:4 parts by volume, respectively.



PATENTED OCT 26 1971

3,615,896



INVENTORS.  
ARTHUR J. BERGER  
ALBERT W. CIZEK, JR.  
RAYMOND J. SIMEON  
BY *Philip Schneider*  
*Don B. Cizek*  
ATTORNEYS

## METAL SURFACE PRIMER

The invention described herein may be manufactured and used by or for the Government of the United States of America for governmental purposes without the payment of any royalties thereon or therefor.

This invention relates to primers for metal surfaces and especially to a tough, thick, adherent, anticorrosive primer for use with nonslip deck coatings.

Laboratory studies and field reports of the U.S. Navy indicate the desirability of applying to clean metal surfaces a tough primer as a base for nonslip deck coatings. Three primers are currently specified in Military Specification MIL-D-23003 (SHIPS) and its Amendment 2 (Formula 117 wash primer; Formula 116, red lead primer; and Formula 84, zinc chromate primer) for priming metal deck surfaces prior to the application of a nonslip deck coating.

In service, the performance of the nonslip deck coatings is found to vary depending on the type of primer used. In most cases, after the nonslip deck coating has worn away or separated from the primer due to poor adhesion, the metal surface starts to corrode rapidly as the primer wears away due to the low impact resistance and inadequate toughness of the latter.

As a result of compatibility studies conducted on two epoxy deck coatings, it has been recommended that only the Formula 117 wash primer be used as a basis for Type II (chemically cured resins, such as epoxies and polyurethanes) coatings of the Military Specification referred to above. Service reports indicate, however, that although the Type II deck coatings show the best adhesion to the Formula 117 wash primer, the primer wears rapidly or is scored readily, allowing corrosion of the steel deck to occur after the deck coating has been worn away. The cause of the rapid wearing and scoring is attributed to the limited thickness, approximately 0.5 mil, of the primer.

An object of this invention is to provide a primer which produces a thicker film having better toughness and abrasion characteristics than the Formula No. 117 wash primer.

Another object is to provide a primer which forms a tough, thick, adherent, anticorrosion film for use with all nonslip deck coatings.

The objects and advantages of this invention are provided by adding a specific moisture-curing, polyurethane resin to the Formula No. 117 wash primer.

Other objects, advantages and novel features of the invention will become apparent from the following detailed description of the invention when considered in conjunction with the accompanying drawing wherein:

The single FIG. is a cross-sectional view of a nonslip deck coating applied to the new primer which is laid on a steel substrate.

The new primer is made by adding a moisture-cured, polyurethane resin to the Formula No. 117 wash primer.

|                                                                    | Pounds per 100 gallons of mixed material | Gallons per 100 gallons of mixed material |
|--------------------------------------------------------------------|------------------------------------------|-------------------------------------------|
| Ingredients of resin component (80 gallons):                       |                                          |                                           |
| Polyvinyl-butylal resin (Note 1).....                              | 56                                       | 6.10                                      |
| Zinc chromate (insoluble type) (Note 2).....                       | 54                                       | 1.78                                      |
| Magnesium-silicate (Type A or B of Specification MIL-M-15173)..... | 8                                        | 0.34                                      |
| Lampblack (Specification TT-L-70).....                             | 0.6                                      | 0.04                                      |
| Butyl alcohol, normal (Spec. TT-B-846).....                        | 125                                      | 18.48                                     |
| Isopropyl alcohol, 99 percent (Notes 3 & 4)...                     | 353                                      | 53.80                                     |
| Water.....                                                         | 15                                       | 1.80                                      |
| Ingredients of acid component (20 gallons):                        |                                          |                                           |
| Phosphoric acid (Class A of Spec. O-P-313) ...                     | 28                                       | 2.0                                       |
| Water.....                                                         | 25                                       | 3.0                                       |
| Isopropyl alcohol, 99 percent (Notes 3 & 4)...                     | 99                                       | 15.0                                      |

1. The resin shall be a polyvinyl partial butylal resin containing only polyvinyl butylal, polyvinyl alcohol, and polyvinyl acetate in the molecule. The resin shall contain 18.0 to 20.0 percent vinyl alcohol, and not more than 1.0 percent of vinyl acetate. A 6 percent solution of the resin in methanol shall

have a viscosity of 12 to 18 centipoises at 20° C. The specific gravity of the resin shall be 1.05 to 1.15.

2. The zinc chromate shall be of an insoluble type, showing an analysis of 16 to 19 percent CrO<sub>3</sub>, and 67 to 72 percent ZnO, and not more than 1 percent water soluble salts.

3. Isopropyl alcohol, 99 percent shall have a specific gravity of 0.785 to 0.790 at 20°/20° C., and a distillation range not greater than 1.5° C., and this range shall include 82.3° C.

4. Ethyl alcohol conforming to Grade III of Specification O-E 10 760 may be substituted for isopropyl alcohol, 99 percent. The isopropyl alcohol (99 percent) and water in the resin component may be replaced by 375 pounds (55.5) gallons of ethyl alcohol. The isopropyl alcohol (99 percent) in the acid component may be replaced by 102 pounds (15.0 gallons) of ethyl alcohol.

15 The formula for the polyurethane resin is provided in U.S. Pat. No. 3,240,618, for "Concrete Form Panels," issued to Charles B. Hemmings on Mar. 15, 1966. A one can urethane system is prepared by reacting under reflux conditions and under inert atmosphere, a diol or triol or any other polyhydroxy compound (polyether polyols, polyester polyols or castor oil), with toluene diisocyanate in a solvent system.

20 The ratio of the isocyanate to polyhydroxy being 2.1/1. The reaction temperature is maintained at reflux and the rate of reaction is controlled by checking the free NCO of the reaction.

25 The urethane prepared above is formulated with solvents to give a 50/50 percent solid content. Antioxidants and driers are also incorporated to give the final urethane coating. The cure of this system is effected by atmosphere moisture. The resin can be obtained commercially from the Spencer Kellogg

30 Division of Textron, Inc. under the designation M80-50CX

The ingredients of the new primer are as follow:

| Part                   | Parts by volume                                | Constituents                                                                                                                       |
|------------------------|------------------------------------------------|------------------------------------------------------------------------------------------------------------------------------------|
| 35 A (Resin Component) | 4                                              | Polyvinyl-butylal resin<br>Zinc chromate<br>Magnesium silicate<br>Lampblack<br>Butyl alcohol, normal<br>Isopropyl alcohol<br>Water |
| 40 B (acid component)  | 1                                              | Phosphoric acid<br>Water<br>Isopropyl alcohol                                                                                      |
| C (resin component)    | 4                                              | M80-50CX polyurethane resin                                                                                                        |
| 45                     | Parts A and B form the constituents of Formula |                                                                                                                                    |

Parts A and B form the constituents of Formula No. 117 wash primer. The mixture is made by adding Part A to Part C 50 and mixing for about 1 minute, then adding Part B and mixing for about 2 minutes more.

The mixture should be made just before it is applied. Application can be accomplished with a standard paint roller.

Test results indicate that the new primer exhibits superior 55 performance as a prime for nonslip deck coatings for the following reasons:

a. After a 1-hour drying period, a film thickness of 2 mils is obtained compared to 0.5 mils for Formula No. 117;

b. The thicker film of the new primer is tough and flexible, 60 as shown by impact resistance tests, and provides excellent corrosion and weathering resistance. Therefore, it provides prolonged protection of the deck prior to the application of the deck-covering compound;

c. The adhesion of Type II nonslip deck coatings to the new 65 primer is excellent.

We claim:

1. A primer for use with nonslip deck coatings of the chemically cured-resin type comprising five parts by volume of wash primer consisting of a mixture of polyvinyl butylal resin, zinc chromate, magnesium silicate, lampblack, butyl alcohol normal, isopropyl alcohol, phosphoric acid and water and four parts by volume of a moisture-cured polyurethane resin.

2. A primer as in claim 1, wherein said polyurethane resin is 70 a polyurethane resin consisting of the reaction product of a polyhydroxy compound with toluene diisocyanate in a solvent

system with antioxidant and drier additives.

3. A primer as in claim 1, wherein four parts by volume of the resin component of said wash primer and four parts by volume of said polyurethane resin are mixed for about 1 minute and then one part by volume of the acid component of said wash primer is mixed in for about 2 minutes more.

4. A primer as in claim 2, wherein four parts by volume of the resin components of said wash primer and four parts by volume of said polyurethane resin are mixed for about 1 minute and then one part by volume of the acid component of said wash primer is mixed in for about 2 minutes.

10

15

20

25

30

35

40

45

50

55

60

65

70

75